

## UNITED STATES PATENT OFFICE

2,033,544

## WAXING AND POLISHING COMPOSITIONS

Anderson W. Ralston and Carl W. Christensen,  
Chicago, Ill., assignors to Armour and Com-  
pany, Chicago, Ill., a corporation of Illinois

No Drawing. Application May 16, 1935,  
Serial No. 21,904

8 Claims. (CL 134—24)

This invention relates to waxing and polishing compounds and it comprises paste-like or fluid compounds composed of wax-like "mixed" ketones and a liquid vehicle therefor.

5 Most of the ordinary waxing and polishing compositions are composed of solid vegetable or animal waxes and a liquid vehicle. The more usual waxes in these compounds are carnauba, beeswax, spermaceti and Montan wax. All of the  
10 animal and vegetable waxes are esters of high molecular weight fatty acids such as myricyl palmitate. For example carnauba wax is mostly myricyl cerotate. Spermaceti is mostly cetyl palmitate, and beeswax is composed of a mixture  
15 of cerotic acid and myricyl palmitate. Montan wax contains a considerable amount of free fatty acids such as arachidic, behenic and lignoceric. These waxes have melting points of from about 42° C. in the case of spermaceti to 80° C. or 90°  
20 C. in the case of carnauba and Montan wax.

When preparing waxing or polishing compositions these waxes are made up into paste-like or somewhat viscous fluid compounds by admixing the wax with a suitable liquid vehicle. In some cases the wax is emulsified in water to yield polishing and waxing compounds which can be spread upon floors and then rubbed down as the water evaporates. In many instances various mixtures of waxes are used in order to obtain the  
30 beneficial physical properties of the separate waxes. All of these vegetable and animal waxes will, when properly applied, adhere rather firmly to a surface and can be worked up to give a high polish.

35 However, waxes of this character are not chemically inert to atmospheric conditions commonly met with. As stated they are all esters. They are not glycerine esters; they are simply the mono esters of higher fatty acids and higher monatomic alcohols. Accordingly they readily undergo hydrolysis in the presence of moisture and they are rather easily oxidized. Wood surfaces polished with these compounds will after a time lose brilliancy. This is because the thin film of wax in immediate contact with atmospheric influences hydrolyzes to a certain extent or oxidizes. This is particularly noticeable in the case of automobile polishes since they are subject to wind and rain. All of these compounds used in ordinary  
45 polishes would show much greater life and resistance to atmospheric influences were it not for the fact that because of their chemical structure they are notoriously susceptible to the action of moisture and air. In other words they are  
50 not at all inert chemically.

We have now set ourselves to the problem of finding a class of compounds which would make very much better polishes for furniture, automobile finishes, floors and the like. We have discovered that a class of compounds known as 5 mixed ketones satisfies the requirement of this art. These mixed ketones have the general molecular structure



wherein R is a carbocyclic or heterocyclic radical 10 and R' is an alkyl radical having at least eleven carbon atoms. These compounds are denoted as mixed ketones in chemical nomenclature for the reason that one of the radicals linked to the carbonyl group is an aryl or heterocyclic radical and the other radical linked to carbonyl is an alkyl group. "Mixed" ketones are not to be confused with mixtures of different ketones.

15 There are a great many compounds coming 20 within the generic scope of our invention and among them are the following.

|                                          | Melting point |
|------------------------------------------|---------------|
| Heptadecyl phenyl ketone                 | 59 °C.        |
| Heptadecyl p-tolyl ketone                | 67 °C. 25     |
| Heptadecyl m-xylyl Ketone                | 39 °C.        |
| Heptadecyl p-xylyl ketone                | 57 °C.        |
| Pentadecyl m-xylyl ketone                | 37 °C.        |
| Pentadecyl p-tolyl ketone                | 60 °C.        |
| p-Methoxyphenyl pentadecyl ketone        | 70.5 °C. 30   |
| p-Ethoxyphenyl pentadecyl ketone         | 69 °C.        |
| Phenyl undecyl ketone                    | 46 °C.        |
| p-Chlorophenyl undecyl ketone            | 57 °C.        |
| p-Methoxyphenyl heptadecyl ketone        | 76 °C.        |
| p-Methoxyphenyl undecyl ketone           | 60 °C. 35     |
| p-Phenoxyphenyl heptadecyl ketone        | 68 °C.        |
| p-Phenoxyphenyl tridecyl ketone          | 53-54° C.     |
| p-Phenoxyphenyl undecyl ketone           | 48-6° C.      |
| p-Nitro phenoxyphenyl heptadecyl ketone  | 177- 9° C. 40 |
| p-Methyl phenoxyphenyl heptadecyl ketone | 177- 9° C.    |
| Alkyl phenones from lard fatty acids.    |               |
| Alpha naphthyl heptadecyl ketone         | 53-4° C.      |
| Alpha naphthyl pentadecyl ketone         | 48° C. 45     |
| Anthracyl heptadecyl ketone (mixtures)   |               |
| Biphenyl heptadecyl ketone               | 108-9° C.     |
| Biphenyl tridecyl ketone                 | 102-103° C.   |
| Biphenyl undecyl ketone                  | 97-98° C.     |
| p-Methyl biphenyl heptadecyl ketone      | 105-6° C. 50  |
| p-Chlor biphenyl heptadecyl ketone       | 96-7° C.      |
| Furyl heptadecyl ketone                  | 52.5-54° C.   |
| Methyl furyl heptadecyl ketone           | 68-9° C.      |
| Dibenzofuryl heptadecyl ketone           | 83-4° C.      |
| Dibenzofuryl undecyl ketone              | 74-5° C.      |

Also ketones wherein the heterocyclic radical is derived from carbazol, thiophene and fluorene.

All of these ketones are wax-like solids. Some of them are old, such as heptadecyl phenyl ketone, commonly called stearophenone, but many of them are new and we have separately described and claimed them in copending applications. All of them have melting points which make them suitable for use in waxing and polishing compositions. Of the compounds listed above those derived from biphenyl are of particularly great interest. It will be noted that these biphenyl ketones all have melting points around 100° C. This is some 20° higher than substances like Montan wax and carnauba wax. Hence polishing compositions using the ketones wherein one of the radicals is biphenyl are particularly useful in polishing surfaces which may be subject to temperatures as high as the boiling point of water in normal use. There are no polishing waxes occurring in nature which display such advantageous properties. Of even greater significance however all of the mixed ketones falling within the general scope of our invention are markedly resistant to heat. And they are of course unaffected by moisture. Hence they cannot hydrolyze and they are substantially inert chemically under all atmospheric conditions ordinarily met with. Automobile polishes made with our ketones show greatly increased life and retain their brilliancy over long periods of time. Moreover our compounds have marked improved adhesion for wood surfaces, the ordinary lacquer automobile finishes and the like.

These ketones can be prepared in well known ways. Generally use is made of the "Friedel Crafts" synthesis. In this, the acid chloride of a higher fatty acid, for example stearyl chloride is reacted with benzene in the presence of aluminum chloride. This will give heptadecyl phenyl ketone. In a similar manner when we wish to make the tolyl compounds we can start with toluene instead of benzene, naphthalene when making the naphthyl compounds, and so on. In a similar way we make ketones containing any desired alkyl radicals by starting with the acid chloride of the corresponding fatty acid. Stearic acid for example is first converted to stearyl chloride in ways well known. Palmityl chloride yields pentadecyl ketones, and from a mixture of lard fatty acids (chiefly oleic acid) we can make corresponding alkyl phenones by converting the fatty acids to their corresponding acid chlorides and then reacting these substances with benzene in the presence of aluminum chloride.

In broad aspects then our invention comprises a wax or polishing composition composed of a mixed ketone as defined above and wherein the alkyl group generally contains eleven or more carbon atoms, admixed with a suitable liquid vehicle. This liquid vehicle can be a solvent for the wax. There are many solvents which we can use. Carbon tetrachloride, acetone and benzene are but a few of the many liquids with which these waxlike ketones are miscible. We can also prepare aqueous emulsions of these ketones by simply emulsifying the ketone in water together with an emulsifying agent. The emulsifying agent can be a soap such as sodium oleate or other emulsifying agent customarily used for emulsifying other waxes such as carnauba in an aqueous vehicle. Advantageously the emulsion is passed through a colloidal mill to homogenize it.

The consistency of our polishing compositions can be a paste-like material, similar to the many different types of semi-solid floor polishes avail-

able to-day, or it can be normally liquid such for example as the liquid type of polish sold for waxing floors. Both of these types generally contain a major quantity of solid waxes and a minor quantity of the liquid vehicle.

We shall now give various examples of ways of practicing our invention.

To prepare a polish of waxlike paste consistency we admix about ten parts of biphenyl heptadecyl ketone with about one part by weight of a solvent such as carbon tetrachloride or benzene. Advantageously the mixture is moderately heated and stirred to incorporate the constituents into a homogeneous mixture. When the mixture cools down we obtain a thick, semi-solid plastic product similar in physical consistency to many of the ordinary semi-solid compositions sold for waxing floors or automobiles. By increasing the quantity of solvent to four parts by weight the resulting composition is a liquid-type polish and can be poured from a can on to a floor and then spread on the floor by means of the usual spreader. Instead of using biphenyl heptadecyl ketone we can of course use any of the ketones described above but ordinarily we prefer to use ketones having melting points of at least 50° C. Advantageously we make compositions containing a mixture of these ketones. For example we prepare a mixture containing about five parts by weight of heptadecyl phenyl ketone, about five parts by weight of biphenyl heptadecyl ketone and about two to eight parts by weight of carbon tetrachloride or benzene. This gives us a composition, which may either be semi-solid or fluid depending upon the quantity of vehicle, in which we obtain the advantageous high melting point of biphenyl heptadecyl ketone and also the desirable properties of heptadecyl phenyl ketone. This latter substance has a somewhat lower melting point and makes it somewhat easier to rub the wax film up to a high gloss. We customarily use mixtures of high and low melting point ketones for this reason. Additionally heptadecyl phenyl ketone is somewhat less expensive than the biphenyl heptadecyl ketone.

As stated we can prepare aqueous emulsions of these ketones, and the emulsions can either be semi-solid paste-like products or liquid, flowable types. Thus for example we emulsify about ten parts by weight of heptadecyl phenyl ketone in about fifteen parts by weight of water containing about one part of sodium oleate as an emulsifier. Of course it is to be understood that other emulsifying agents can be used and in this respect we follow the general practice customarily employed in emulsifying oils and waxes in water. In the case of emulsions the proportions can vary over a wide range, such that the final composition will contain from about 10 to 80 percent of ketone.

It is of course to be understood that we can use many mixtures of the ketones described above. We can for example first melt together equal parts by weight of pentadecyl parafolyl ketone, phenyl undecyl ketone and alphanaphthyl pentadecyl ketone. Or we can prepare basic wax mixtures containing largely ketones of the biphenyl series associated with smaller amounts of ketones of the phenyl or naphthyl series.

In the customary practice of our invention however we prefer to use the less costly phenyl, naphthyl, and biphenyl compounds. We have, however, disclosed a number of ketones wherein one of the radicals is heterocyclic. These are the furyl compounds, the carbazols, the thiophenes

and the fluoryls. We have done this to indicate the generic characteristics of our invention.

Although we have referred more specifically to the use of our ketones as the major wax constituent in our compositions, we can of course admix our ketones with other kinds of polishing waxes. For example we can prepare a wax composed of about equal parts of biphenyl heptadecyl ketone and carnauba wax and then emulsify this mixture in water or incorporate a volatile solvent. Instead of using carnauba we can use beeswax, Montan wax and any of the other waxes hitherto used in compositions of this character. The proportions can vary over a wide range and the addition of as little as one part of biphenyl heptadecyl ketone to eight parts of carnauba or Montan wax is beneficial, and the resulting composition when taken up in a liquid vehicle, is improved by the presence of the ketone. Thus it will be apparent that our invention can be modified over a wide range.

Practically all of the commercial waxing and polishing compositions are made up in such proportions that the wax material therein constitutes the major quantity of the composition. In consistency, these products vary from paste-like materials to somewhat viscous flowable liquids. All volatile solvent type compositions in paste-like cakes contain a major quantity of a solid constituent but some of the liquid types, namely the emulsions may contain sixty percent or more of aqueous vehicle. Accordingly in the appended claims we do not wish to limit ourselves, in the case of emulsions, to any particular quantities of aqueous vehicle and wax.

As stated, many of the ketones which we use are new materials. In our copending applications we have described and claimed them as such. In our copending application Serial Number 17,873, filed April 23, 1935, we have claimed the mixed 40 phenoxy phenyl alkyl ketones, in our copending application Serial Number 17,874, filed April 23, 1935, we have claimed the mixed diphenyl alkyl ketones, in our copending application Serial Number 17,875, filed April 23, 1935, we have claimed the 45

mixed furyl alkyl ketones, and in our application Serial Number 48,940, filed November 8, 1935 as a division of Serial Number 17,875, we have claimed the benzofuryl alkyl ketones.

Having thus described our invention what we 5 claim is:

1. A composition for waxing or polishing comprising a major quantity of a wax constituent including a ketone, and a minor quantity of a liquid vehicle for the wax constituent, the ketone 10 having the general structure



wherein R is a radical chosen from the group consisting of carbocyclic and heterocyclic radicals, 15 and R' is an alkyl radical containing at least eleven carbon atoms.

2. The composition as in claim one wherein the liquid vehicle is a volatile solvent.

3. A composition for waxing or polishing comprising a major quantity of a wax constituent including a waxy aralkyl ketone and a minor quantity of a liquid vehicle.

4. The composition as in claim three wherein 25 the liquid vehicle is a volatile solvent.

5. The composition as in claim three wherein the ketone is a waxy biphenyl-alkyl ketone.

6. A composition for waxing or polishing comprising an aqueous emulsion of a ketone having 30 the general structure



wherein R is a radical chosen from the group consisting of carbocyclic and heterocyclic radicals, 35 and R' is an alkyl radical containing at least eleven carbon atoms.

7. A composition for waxing or polishing comprising an aqueous emulsion of a waxy aralkyl ketone.

8. The composition as in claim seven wherein 40 the ketone is a waxy biphenyl-alkyl ketone.

ANDERSON W. RALSTON.  
CARL W. CHRISTENSEN. 45